

# United States Patent [19]

Michalko et al.

[11]

4,226,639

[45]

Oct. 7, 1980

[54] **SILICA GUARD BED FOR ADSORBENT  
USED IN AN AQUEOUS SYSTEM**

[75] Inventors: **Edward Michalko, Hemet, Calif.;  
Armand J. deRosset, Clarendon Hills,  
Ill.**

[73] Assignee: **UOP Inc., Des Plaines, Ill.**

[21] Appl. No.: **42,479**

[22] Filed: **May 25, 1979**

[51] Int. Cl.<sup>3</sup> ..... **C13D 3/14**

[52] U.S. Cl. ..... **127/46 A; 127/46 B;  
127/55; 536/1; 210/670; 210/690**

[58] **Field of Search** ..... **127/46 R, 46 A, 46 B,  
127/55; 210/27, 32, 36, 38, 40; 536/1**

## [56] References Cited

### U.S. PATENT DOCUMENTS

4,014,711 3/1977 Odawara et al. ..... 127/46 B  
4,157,267 6/1979 Odawara et al. ..... 127/46 A

Primary Examiner—Michael S. Marcus

*Attorney, Agent, or Firm*—James R. Hoatson, Jr.; Louis A. Morris; William H. Page, II

[57]

## ABSTRACT

A process for separating a component from a feed mixture comprising an aqueous solution of a mixture of different components, such as a mixture of saccharides, in which the mixture is contacted with an adsorbent comprising a crystalline aluminosilicate which selectively adsorbs a component from the feed mixture. The adsorbed component is then recovered by contacting the adsorbent with a desorbent material such as water to effect the desorption of the adsorbed component from the adsorbent. There is an undesirable tendency for the silicon constituent of the crystalline aluminosilicate to dissolve in the aqueous system. The improvement to the process comprises contacting the desorbent, and/or the feed mixture, with a bed of silica gel prior to contacting the feed mixture with the adsorbent. This effects a substantial reduction in the undesirable dissolution.

6 Claims, No Drawings

## SILICA GUARD BED FOR ADSORBENT USED IN AN AQUEOUS SYSTEM

### BACKGROUND OF THE INVENTION

#### 1. Field of the Invention

The field of art to which this invention pertains is solid-bed adsorptive separation. More specifically, the invention relates to an improved process for separating a component from a mixture comprising an aqueous solution of a mixture of different components which process employs an adsorbent comprising a crystalline aluminosilicate which selectively adsorbs a component from the feed mixture.

#### 2. Description of the Prior Art

It is known in the separation art that certain crystalline aluminosilicates, referred to as zeolites, can be used in the separation of a component from an aqueous solution of a mixture of different components. For example, adsorbents comprising crystalline aluminosilicate are used in the method described in U.S. Pat. No. 4,014,711 to separate fructose from a mixture of sugars in aqueous solution including fructose and glucose.

It is also known that crystalline aluminosilicates or zeolites are used in adsorption processing in the form of 25 agglomerates having high physical strength and attrition resistance. Methods for forming the crystalline powders into such agglomerates include the addition of an organic binder, generally a clay comprising silicon dioxide and aluminum oxide to the high purity zeolite powder in wet mixture. The blended clay zeolite mixture is extruded into cylindrical type pellets or formed into beads which are subsequently calcined in order to convert the clay to an amorphous binder of considerable mechanical strength. As binders, clays of the kaolin 30 type are generally used.

Zeolite crystals have long been known to have the property of gradually disintegrating as a result of continuous contact with water. It may be related to the 40 surface migration and interaction between the charges of ions on the zeolite surface and in solution. In any event, the zeolite disintegration has been observed as a silicon presence in the solution in contact with the zeolite.

We have discovered an improvement to an aqueous 45 separation process which minimizes the dissolution and disintegration of the adsorbent.

### SUMMARY OF THE INVENTION

It is accordingly a broad objective of our invention to 50 provide an improvement to a process for the separation of a component from a feed mixture comprising different components in aqueous solution, by contacting said mixture with an adsorbent comprising a crystalline aluminosilicate, so as to minimize the dissolution and disintegration of the crystalline aluminosilicate.

In brief summary, our invention is, in one embodiment, a process for the separation of a component from a feed mixture comprising an aqueous solution of a mixture of components by contacting the solution with an adsorbent comprising a crystalline aluminosilicate exhibiting an adsorptive selectivity towards the component. The component is thereby selectively adsorbed from the mixture, and the adsorbed component is thereafter recovered by elution with a desorbent. The silicon constituent of the crystalline aluminosilicate tends to dissolve in the solution resulting in the undesirable disintegration of the crystalline aluminosilicate. The im-

provement comprises contacting the feed mixture and/or desorbent with a bed of silica gel prior to contacting the feed mixture and/or desorbent with the adsorbent. This effects a substantial reduction in the extent of dissolution of the silicon constituent and the extent of the disintegration of the crystalline aluminosilicate in the adsorbent.

Other objectives and embodiments of our invention encompass details about feed mixtures, adsorbents, desorbent materials and operating conditions, all of which are hereinafter disclosed in the following discussion of each of the facets of the present invention.

### DESCRIPTION OF THE INVENTION

15 At the outset, the definitions of various terms used throughout the specification will be useful in making clear the operation, objects and advantages of our process.

20 A feed mixture is a mixture containing one or more extract components and one or more raffinate components to be separated by our process. The term "feed stream" indicates a stream of a feed mixture which passes to the adsorbent used in the process.

An "extract component" is a component that is more 25 selectively adsorbed by the adsorbent while a "raffinate component" is a component that is less selectively adsorbed. The term "desorbent material" shall mean generally a material capable of desorbing an extract component. The term "desorbent stream" or "desorbent input stream" indicates the stream through which desorbent material passes to the adsorbent. The term "raffinate stream" or "raffinate output stream" means a stream through which a raffinate component is removed from the adsorbent. The composition of the raffinate stream can vary from essentially 100% desorbent material to essentially 100% raffinate components. The term "extract stream" or "extract output stream" shall mean a stream through which an extract material which has 30 been desorbed by a desorbent material is removed from the adsorbent. The composition of the extract stream, likewise, can vary from essentially 100% desorbent material to essentially 100% extract components. At least a portion of the extract stream and preferably at least a portion of the raffinate stream from the separation process are passed to separation means, typically fractionators or evaporators, where at least a portion of desorbent material is separated to produce an extract product and a raffinate product. The terms "extract product" and "raffinate product" mean products produced by the process containing, respectively, an extract component and a raffinate component in higher concentrations than those found in the extract stream and the raffinate stream.

The term "selective pore volume" of the adsorbent is 35 defined as the volume of the adsorbent which selectively adsorbs an extract component from the feed mixture. The term "non-selective void volume" of the adsorbent is the volume of the adsorbent which does not selectively retain an extract component from the feed mixture. This volume includes the cavities of the adsorbent which contain no adsorptive sites and the interstitial void spaces between adsorbent particles. The selective pore volume and the non-selective void volume are 40 generally expressed in volumetric quantities and are of importance in determining the proper flow rates of fluid required to be passed into an operational zone for efficient operations to take place for a given quantity of

adsorbent. When adsorbent "passes" into an operational zone (hereinafter defined and described) employed in one embodiment of this process, its non-selective void volume, together with its selective pore volume, carries fluid into that zone. The non-selective void volume is utilized in determining the amount of fluid which should pass into the same zone in a counter-current direction to the adsorbent to displace the fluid present in the non-selective void volume. If the fluid flow rate passing into a zone is smaller than the non-selective void volume rate of adsorbent material passing into that zone, there is a net entrainment of liquid into the zone by the adsorbent. Since this net entrainment is a fluid present in non-selective void volume of the adsorbent, it in most instances comprises less selectively retained feed components. The selective pore volume of an adsorbent can in certain instances adsorb portions of raffinate material from the fluid surrounding the adsorbent since in certain instances there is competition between extract material and raffinate material for adsorptive sites within the selective pore volume. If a large quantity of raffinate material with respect to extract material surrounds the adsorbent, raffinate material can be competitive enough to be adsorbed by the adsorbent.

The so-called "simple sugars" are classified as monosaccharides and are those sugars which upon hydrolysis do not break down into smaller simpler sugars. One may further classify monosaccharides as aldoses or ketoses, depending upon whether they are hydroxy aldehydes or hydroxy ketones, and by the number of carbon atoms in the molecule. Most common and well known are probably the hexoses. Common ketohexoses are fructose (levulose) and sorbose; common aldochexoses are glucose (dextrose), mannose and galactose. The term "oligosaccharides" as commonly understood in the art and as used herein means simple polysaccharides containing a known number of constituent monosaccharide units. An oligosaccharide that breaks up upon hydrolysis into two monosaccharide units is called a disaccharide, examples being sucrose, maltose and lactose. Those giving three such units are trisaccharides, of which raffinose and melezitose are examples. Di-, tri- and tetra-saccharides comprise practically all of the oligosaccharides. The term "polysaccharide" includes oligosaccharides but usually it refers to carbohydrate materials of much higher molecular weight, namely, those that are capable of breaking up on hydrolysis into a large number of monosaccharide units. Typical polysaccharides are starch, glycogen, cellulose and pentosans.

Feed mixtures which can be charged to the process of our invention may, for example, be aqueous solutions of one or more aldoses and one or more ketoses or one or more monosaccharides and one or more oligosaccharides. The concentration of solids in the solutions may range from about 0.5 wt. % to about 50 wt. % or more, but preferably will be from about 5 to about 35 wt. %. Starch syrups such as corn syrup are examples of feed mixtures which can be charged to our process. Such syrups are produced by the partial hydrolysis of starch generally in the presence of mineral acids or enzymes. Corn syrup produced in this manner will typically contain 25 to 75 wt. % solids comprising 90 to 95% glucose and 5 to 10% maltose and higher oligosaccharides. A portion of the glucose in this corn syrup may be isomerized with an isomerizing enzyme to produce a high-fructose corn syrup, typically comprising 40-45% fructose, 50-55% glucose and 5-10% oligosaccharides,

which can also be charged to our process. The pH of the aqueous solution comprising the feed mixture may be from about 5.5 to about 7.5

Desorbent materials used in various prior art adsorptive separation processes vary depending upon such factors as the type of operation employed. In the swing-bed system in which the selectively adsorbed feed component is removed from the adsorbent by a purge stream, desorbent selection is not as critical and desorbent material comprising gaseous hydrocarbons such as methane, ethane, etc., or other types of gases such as nitrogen or hydrogen, may be used at elevated temperatures or reduced pressures, or both, to effectively purge the adsorbed feed component from the adsorbent. However, in adsorptive separation processes which are generally operated continuously at appropriate pressures and temperatures to insure liquid phase, the desorbent material must be judiciously selected to satisfy many criteria. First, the desorbent material should displace an extract component from the adsorbent with reasonable mass flow rates without itself being so strongly adsorbed as to unduly prevent an extract component from displacing the desorbent material in a following adsorption cycle. Expressed in terms of the selectivity (hereinafter discussed in more detail), it is preferred that the adsorbent be more selective for all of the extract components with respect to a raffinate component than it is for the desorbent material with respect to a raffinate component. Secondly, desorbent material must be compatible with the particular adsorbent and the particular feed mixture. More specifically, they must not reduce or destroy the critical selectivity of the adsorbent for an extract component with respect to a raffinate component. Additionally, desorbent materials should not chemically react with or cause a chemical reaction of either an extract component or a raffinate component. Both the extract stream and the raffinate stream are typically removed from the adsorbent in admixture with desorbent material and any chemical reaction involving a desorbent material and an extract component or a raffinate component would reduce the purity of the extract product or the raffinate product or both. Since both the raffinate stream and the extract stream typically contain desorbent materials, desorbent materials should additionally be substances which are easily separable from the feed mixture that is passed into the process. Without a method of separating at least a portion of the desorbent material present in the extract stream and the raffinate stream, the concentration of an extract component in the extract product and the concentration of a raffinate component in the raffinate product would not be very high, nor would the desorbent material be available for reuse in the process. It is contemplated that at least a portion of the desorbent material will be separated from the extract and the raffinate streams by distillation or evaporation but other separation methods such as reverse osmosis may also be employed alone or in combination with distillation or evaporation. Since the raffinate and extract products are foodstuffs intended for human consumption, desorbent materials should also be non-toxic. Finally, desorbent materials should also be materials which are preferably readily available and therefore reasonable in cost.

We have found that water having a pH of from about 5.5 to about 7.5 satisfies these criteria and is a suitable and preferred desorbent material for our process. The pH of the desorbent material is important because adsorption of a component by the adsorbent, removal of a

raffinate stream, desorption of the component from the adsorbent and removal of an extract stream all typically occur in the presence of desorbent material. If the desorbent material is too acidic or too alkaline, chemical reactions of the components are promoted and reaction products are produced that can reduce the yield purity of either the extract or raffinate product, or both.

Water pH does of course vary widely depending upon the source of the water in addition to other factors. Methods of maintaining and controlling a desired water pH are, however, well known to those skilled in the art of water treating. Such methods generally comprise adding an alkaline compound such as sodium hydroxide or an acid compound such as hydrochloric acid to the water in amounts as necessary to achieve and maintain the desired pH.

The prior art has recognized that certain characteristics of adsorbents are highly desirable, if not absolutely necessary, to the successful operation of a selective adsorption process. Such characteristics are equally important to this process. Among such characteristics are: adsorptive capacity for same volume of an extract component per volume of adsorbent; the selective adsorption of an extract component with respect to a raffinate component and the desorbent material; and sufficiently fast rates of adsorption and desorption of an extract component to and from the adsorbent. Capacity of the adsorbent for adsorbing a specific volume of an extract component is, of course, a necessity; without such capacity the adsorbent is useless for adsorptive separation. Furthermore, the higher the adsorbent's capacity for an extract component the better is the adsorbent. Increased capacity of a particular adsorbent makes it possible to reduce the amount of adsorbent needed to separate an extract component of known concentration contained in a particular charge rate of feed mixture. A reduction in the amount of adsorbent required for a specific adsorptive separation reduces the cost of the separation process. It is important that the good initial capacity of the adsorbent be maintained during actual use in the separation process over some economically desirable life. The second necessary adsorbent characteristic is the ability of the adsorbent to separate components of the feed; or, in other words, that the adsorbent possess adsorptive selectivity, (B), for one component as compared to another component.

Relative selectivity can be expressed not only for one feed component as compared to another but can also be expressed between any feed mixture component and the desorbent material. The selectivity, (B), as used throughout this specification is defined as the ratio of the two components of the adsorbed phase over the ratio of the same two components in the unadsorbed phase at equilibrium conditions. Relative selectivity is shown as Equation 1 below:

$$\text{Selectivity} = (B) = \frac{[\text{vol. percent } C/\text{vol. percent } D]_A}{[\text{vol. percent } C/\text{vol. percent } D]_U} \quad \text{Equation 1}$$

where C and D are two components of the feed represented in volume percent and the subscripts A and U represent the adsorbed and unadsorbed phases respectively. The equilibrium conditions were determined when the feed passing over a bed of adsorbent did not change composition after contacting the bed of adsorbent. In other words, there was no net transfer of material occurring between the unadsorbed and adsorbed phases. Where selectivity of two components appro-

aches 1.0, there is no preferential adsorption of one component by the adsorbent with respect to the other: they are both adsorbed (or non-adsorbed) to about the same degree with respect to each other. As the (B) becomes less than or greater than 1.0, there is a preferential adsorption by the adsorbent for one component with respect to the other. When comparing the selectivity by the adsorbent of one component C over component D, a (B) larger than 1.0 indicates preferential adsorption of component C within the adsorbent. A (B) less than 1.0 would indicate that component D is preferentially adsorbed leaving an unadsorbed phase richer in component C and an adsorbed phase richer in component D. Ideally, desorbent materials should have a selectivity equal to about 1 or slightly less than 1 with respect to all extract components so that all of the extract components can be desorbed as a class with reasonable flow rates of desorbent material and so that extract components can displace desorbent material in a subsequent adsorption step. While separation of an extract component from a raffinate component is theoretically possible when the selectivity of the adsorbent for the extract component with respect to the raffinate component is greater than 1.0, it is preferred that such selectivity be greater than 2.0. Like relative volatility, the higher the selectivity the easier the separation is to perform. Higher selectivities permit a smaller amount of adsorbent to be used. The third important characteristic is the rate of exchange of the extract component of the feed mixture material or, in other words, the relative rate of desorption of the extract component. This characteristic relates directly to the amount of desorbent material that must be employed in the process to recover the extract component from the adsorbent; faster rates of exchange reduce the amount of desorbent material needed to remove the extract component and therefore permit a reduction in the operating cost of the process. With faster rates of exchange, less desorbent material has to be pumped through the process and separated from the extract stream for reuse in the process.

Adsorbents to be used in the process of this invention will comprise specific crystalline aluminosilicates or molecular sieves. Particular crystalline aluminosilicates encompassed by the present invention include crystalline aluminosilicate cage structures in which the alumina and silica tetrahedra are intimately connected in an open three dimensional network to form cage-like structures with windowlike pores of about 8 Å free diameter. The tetrahedra are cross-linked by the sharing of oxygen atoms with spaces between the tetrahedra occupied by water molecules prior to partial or total dehydration of this zeolite. The dehydration of the zeolite results in crystals interlaced with cells having molecular dimensions and thus the crystalline aluminosilicates are often referred to as "molecular sieves", particularly when the separation which they effect is dependent essentially upon differences between the sizes of the feed molecules as, for instance, when smaller normal paraffin molecules are separated from larger iso-paraffin molecules by using a particular molecular sieve.

In hydrated form, the crystalline aluminosilicates used in the process of our invention generally encompass those zeolites represented by the Formula 1 below:

## Formula 1



where "M" is a cation which balances the electrovalence of the aluminum-centered tetrahedra and which is generally referred to as an exchangeable cationic site, "n" represents the valence of the cation, "w" represents the moles of  $SiO_2$ , and "y" represents the moles of water. The generalized cation "M" may be monovalent, 10 divalent or trivalent or mixtures thereof.

The prior art has generally recognized that adsorbents comprising X and Y zeolites can be used in certain adsorptive separation processes. These zeolites are described and defined in U.S. Pat. Nos. 2,882,244 and 15 3,120,007 respectively incorporated herein by reference thereto. The X zeolite in the hydrated or partially hydrated form can be represented in terms of mole oxides as shown in Formula 2 below:

## Formula 2



where "M" represents at least one cation having a valence of not more than 3, "n" represents the valence of "M", and "y" is a value up to about 9 depending upon the identity of "M" and the degree of hydration of the crystal. As noted from Formula 2 the  $SiO_2/Al_2O_3$  mole ratio of X zeolite is  $2.5 \pm 0.5$ . The cation "M" may be 30 one or more of a number of cations such as a hydrogen cation, an alkali metal cation, or an alkaline earth cation, or other selected cations, and is generally referred to as an exchangeable cationic site. As the X zeolite is initially prepared, the cation "M" is usually predominately 35 sodium, that is, the major cation at the exchangeable cationic sites is sodium and the zeolite is therefore referred to as a sodium-X zeolite. Depending upon the purity of the reactants used to make the zeolite, other cations mentioned above may be present, however, as 40 impurities. The Y zeolite in the hydrated or partially hydrated form can be similarly represented in terms of mole oxides as in Formula 3 as follows:

## Formula 3



where "M" is at least one cation having a valence not more than 3, "n" represents the valence of "M", "w" is 50 a value greater than about 3 up to about 6, and "y" is a value up to about 9 depending upon the identity of "M" and the degree of hydration of the crystal. The  $SiO_2/Al_2O_3$  mole ratio for Y zeolites can thus be from about 3 to about 6. Like the X zeolite, the cation "M" may be one or more of a variety of cations but, as the Y zeolite is initially prepared, the cation "M" is also usually predominantly sodium. A Y zeolite containing predominantly sodium cations at the exchangeable cationic sites is therefore referred to as a sodium-Y 60 zeolite.

Cations occupying exchangeable cationic sites in the zeolite may be replaced with other cations by ion exchange methods well known to those having ordinary skill in the field of crystalline aluminosilicates. Such 65 methods are generally performed by contacting the zeolite or an adsorbent material containing the zeolite with an aqueous solution of the soluble salt of the cation

or cations desired to be placed upon the zeolite. After the desired degree of exchange takes place, the sieves are removed from the aqueous solution, washed and dried to a desired water content. By such methods, the sodium cations and any nonsodium cations which might be occupying exchangeable sites as impurities in a sodium-X or sodium-Y zeolite can be partially or essentially completely replaced with other cations. It is preferred that the zeolite used in the process of our invention contain cations at exchangeable cationic sites selected from the group consisting of the alkali metals and the alkaline earth metals.

Typically, adsorbents used in separative processes contain zeolite crystals and amorphous material. The zeolite will typically be present in the adsorbent in amounts ranging from about 75 wt. % to about 98 wt. % based on volatile free composition. Volatile free compositions are generally determined after the adsorbent has been calcined at 900° C. in order to drive off all volatile matter. The remainder of the adsorbent will generally be amorphous material such as silica, or silica-alumina mixtures or compounds, such as clays, which material is present in intimate mixture with the small particles of the zeolite material. This amorphous material may be an adjunct of the manufacturing process for zeolite (for example, intentionally incomplete purification of either zeolite during its manufacture), or it may be added to relatively pure zeolite, but in either case its usual purpose is as a binder to aid in forming or agglomerating the hard crystalline particles of the zeolite. Normally, the adsorbent will be in the form of particles such as extrudates, aggregates, tablets, macrospheres or granules having a desired particle size range. The adsorbent used in our process will preferably have a particle size range of about 16-40 mesh (Standard U.S. Mesh). Examples of suitable zeolites employed in our process, either as is or after cation exchange, are "Molecular Sieves 13X" and "SK-40", both of which are available from the Linde Company, Tonawanda, New York. The first material of course contains X zeolite while the latter material contains Y zeolite. We have found that X or Y zeolites possess the selectivity requirement and other necessary requirements previously discussed and are therefore suitable for use in our process.

The question arises, particularly when the amorphous binders material in the adsorbent comprises silica or silica-alumina, whether the source of the dissolved silicon in the solution in contact with the adsorbent is the zeolite or the binder material. We have found that the primary source of the silicon is in fact the zeolite. The removal of the silicon from the crystalline aluminosilicate via its dissolution in the aqueous solution causes collapse of the crystalline structure which renders the adsorbent ineffective for use in the process of this invention. However, silicon is also leached from the silica or silica/alumina binder, and its dissolution causes generation of fine particles of zeolite which can be mechanically lost from the bed, or may accumulate at critical points in the flow scheme and cause pressure drop.

In accordance with our invention, prior to contacting the feed mixture and/or desorbent of the process of our invention with the adsorbent, the feed mixture and/or desorbent is contacted with a bed, sometimes referred to as a guard bed, of silica gel. The silica gel comprises an amorphous solid material having  $SiO_2$  as the basic chemical composition. The guard bed will preferably comprise a dense compact fixed bed of particles of the silica gel.

We have determined that only silica gel is effective for use in the guard bed. For example, use of sodium silicate in the guard bed will not prevent the dissolution of the silicon constituent of the crystalline aluminosilicate in the adsorbent. We have developed the hypothesis set forth in the following paragraph to account for the difference in effectiveness between the sodium silicate and the silica gel.

When silica gel is contacted with water, a small but finite level of solubility is observed. The solubility increases with temperature. When the silica gel becomes hydrated and solubilized, the solute is referred to as silicic acid, wherein the silicon atom is tetrahedrally coordinated to 4 hydroxyl groups. In zeolites also, the silicon atom is linked by bonding to 4 oxygen atoms (ions) or, in other words, is tetrahedrally coordinated. In the case of sodium silicate, the silicon atom is normally linked to or coordinated with 6, rather than 4, hydroxyl ligands and is thus referred to as being in hexa-coordination. We have thus hypothesized that the coordination level of the soluble silica species must match that of the silica contained in the zeolite that we wish to protect. The same hypothesis is applicable to protection of the silica or silica/alumina binders with tetrahedrally coordinated silica, since these binders also comprise tetrahedrally coordinated silica structure.

The feed mixture or desorbent passes from the guard bed to the adsorbent. The adsorbent may be employed in the form of a dense compact fixed bed which is alternatively contacted with the feed mixture and desorbent materials. In the simplest embodiment of the invention, the adsorbent is employed in the form of a single static bed in which case the process is only semi-continuous. In another embodiment, a set of two or more static beds may be employed in fixed-bed contacting with appropriate valving so that the feed mixture is passed through one or more adsorbent beds while the desorbent materials can be passed through one or more of the other beds in the set. The flow of feed mixture and desorbent materials may be either up or down through the desorbent. Any of the conventional apparatus employed in static bed fluid-solid contacting may be used.

Counter-current moving-bed or simulated moving-bed counter-current flow systems, however, have a much greater separation efficiency than fixed adsorbent bed systems and are therefore preferred for use in our separation process. In the moving-bed or simulated moving-bed processes, the adsorption and desorption operations are continuously taking place which allows both continuous production of an extract and a raffinate stream and the continual use of feed and desorbent streams. One preferred embodiment of this process utilizes what is known in the art as the simulated moving-bed counter-current flow system. The operating principles and sequence of such a flow system are described in U.S. Pat. No. 2,985,589 incorporated herein by reference thereto. In such a system, it is the progressive movement of multiple liquid access points down an adsorbent chamber that simulates the upward movement of adsorbent contained in the chamber. Only four of the access lines are active at any one time; the feed input stream, desorbent inlet stream, raffinate outlet stream, and extract outlet stream access lines. Coincident with this simulated upward movement of the solid adsorbent is the movement of the liquid occupying the void volume of the packed bed of adsorbent. So that counter-current contact is maintained, a liquid flow down the adsorbent chamber may be provided by a

5 pump. As an active liquid access point moves through a cycle, that is, from the top of the chamber to the bottom, the chamber circulation pump moves through different zones which require different flow rates. A programmed flow controller may be provided to set and regulate these flow rates.

10 The active liquid access points effectively divided the adsorbent chamber into separate zones, each of which has a different function. In this embodiment of our process, it is generally necessary that three separate operational zones be present in order for the process to take place although in some instances an optional fourth zone may be used.

15 The adsorption zone, zone 1, is defined as the adsorbent located between the feed inlet stream and the raffinate outlet stream. In this zone, the feed stock contacts the adsorbent, an extract component is adsorbed, and a raffinate stream is withdrawn. Since the general flow through zone 1 is from the feed stream which passes into the zone to the raffinate stream which passes out of the zone, the flow in this zone is considered to be a downstream direction when proceeding from the feed inlet to the raffinate outlet streams.

20 Immediately upstream with respect to fluid flow in zone 1 is the purification zone, zone 2. The purification zone is defined as the adsorbent between the extract outlet stream and the feed inlet stream. The basic operations taking place in zone 2 are the displacement from the non-selective void volume of the adsorbent of any raffinate material carried into zone 2 by the shifting of adsorbent into this zone and the desorption of any raffinate material adsorbed within the selective pore volume of the adsorbent or adsorbed on the surfaces of the adsorbent particles. Purification is achieved by passing 25 a portion of extract stream material leaving zone 3 into zone 2 at zone 2's upstream boundary, the extract outlet stream, to effect the displacement of raffinate material. The flow of material in zone 2 is in a downstream direction from the extract outlet stream to the feed inlet stream.

30 Immediately upstream of zone 2 with respect to the fluid flowing in zone 2 is the desorption zone or zone 3. The desorption zone is defined as the adsorbent between the desorbent inlet and the extract outlet stream. The function of the desorption zone is to allow a desorbent material which passes into this zone to displace the extract component which was adsorbed upon the adsorbent during a previous contact with feed in zone 1 in a prior cycle of operation. The flow of fluid in zone 35 is essentially in the same direction as that of zones 1 and 2.

35 In some instances, an optional buffer zone, zone 4, may be utilized. This zone, defined as the adsorbent between the raffinate outlet stream and the desorbent inlet stream, if used, is located immediately upstream with respect to the fluid flow to zone 3. Zone 4 would be utilized to conserve the amount of desorbent utilized in the desorption step since a portion of the raffinate stream which is removed from zone 1 can be passed into zone 4 to displace desorbent material present in that zone out of that zone into the desorption zone. Zone 4 will contain enough adsorbent so that raffinate material present in the raffinate stream passing out of zone 1 and into zone 4 can be prevented from passing into zone 3 thereby contaminating extract stream removed from zone 3. In the instances in which the fourth operational zone is not utilized the raffinate stream passed from zone 1 to zone 4 must be carefully monitored in order

that the flow directly from zone 1 to zone 3 can be stopped when there is an appreciable quantity of raffinate material present in the raffinate stream passing from zone 1 into zone 3 so that the extract outlet stream is not contaminated.

A cyclic advancement of the input and output streams through the fixed bed of adsorbent can be accomplished by utilizing a manifold system in which the valves in the manifold are operated in a sequential manner to effect the shifting of the input and output streams, thereby allowing a flow of fluid with respect to solid adsorbent in a counter-current manner. Another mode of operation which can effect the counter-current flow of solid adsorbent with respect to fluid involves the use of a rotating disc valve in which the input and output streams are connected to the valve and the lines through which feed input, extract output, desorbent input and raffinate output streams pass are advanced in the same direction through the adsorbent bed. Both the manifold arrangement and disc valve are known in the art. Specifically, rotary disc valves which can be utilized in this operation can be found in U.S. Pat. Nos. 3,040,777 and 3,422,848. Both of the aforementioned patents disclose a rotary type connection valve in which the suitable advancement of the various input and output streams from fixed sources can be achieved without difficulty.

In many instances, one operational zone will contain a much larger quantity of adsorbent than some other operational zone. For instance, in some operations the buffer zone can contain a minor amount of adsorbent as compared to the adsorbent required for the adsorption and purification zones. It can also be seen that in instances in which desorbent is used which can easily desorb extract material from the adsorbent that a relatively small amount of adsorbent will be needed in a desorption zone as compared to the adsorbent needed in the buffer zone or adsorption zone or purification zone or all of them. Since it is not required that the adsorbent be located in a single column, the use of multiple chambers or a series of columns is within the scope of the invention.

It is not necessary that all of the input or output streams be simultaneously used, and in fact, in many instances some of the streams can be shut off while others effect an input or output of material. The apparatus which can be utilized to effect the process of this invention can also contain a series of individual beds connected by connecting conduits upon which are placed input or output taps to which the various input or output streams can be attached and alternately and periodically shifted to effect continuous operation. In some instances, the connecting conduits can be connected to transfer taps which during the normal operations do not function as a conduit through which material passes into or out of the process.

It is contemplated that at least a portion of the extract output stream will pass into a separation means wherein at least a portion of the desorbent material can be separated to produce an extract product containing a reduced concentration of desorbent material. Preferably, but not necessary to the operation of the process, at least a portion of the raffinate output stream will also be passed to a separation means wherein at least a portion of the desorbent material can be separated to produce a desorbent stream which can be reused in the process and a raffinate product containing a reduced concentration of desorbent material. The separation means will

typically be a fractionation column or an evaporator, the design and operation of either being well known to the separation art.

Reference can be made to D. B. Broughton U.S. Pat. No. 2,985,589, and to a paper entitled "Continuous Adsorptive Processing—A New Separation Technique" by D. B. Broughton presented at the 34th Annual Meeting of the Society of Chemical Engineers at Tokyo, Japan, on Apr. 2, 1969, for further explanation of the simulated moving-bed counter-current process flow scheme.

Although both liquid and vapor phase operations can be used in many adsorptive separation processes, liquid phase operation is required for this process because of the lower temperature requirements and because of the higher yields of extract product that can be obtained with liquid-phase operation over those obtained with vapor-phase operation. Adsorption conditions will include a temperature range of from about 20° C. to about 100° C. and a pressure range of from about atmospheric to about 500 psig. with from about atmospheric to about 250 psig. being more preferred to insure liquid phase. We have found that our invention is most effective at temperatures below about 65° C. Desorption conditions will include the same range of temperatures and pressures as used for adsorption conditions.

The size of the units which can utilize the process of this invention can vary anywhere from those of pilot-plant scale (see for example our assignee's U.S. Pat. No. 3,706,812) to those of commercial scale and can range in flow rates from as little as a few cc an hour up to many thousands of gallons per hour.

A dynamic testing apparatus is employed to test various sources of added silica with a particular adsorbent to measure the extent of silicon loss from the adsorbent when contacted with an aqueous feed. The apparatus consists of an adsorbent chamber of approximately 70 cc volume having inlet and outlet portions at opposite ends of the chamber. The chamber is contained within a temperature control means and, in addition, pressure control equipment is used to operate the chamber at a constant predetermined pressure. Means are provided to prepare the aqueous feed. When the effect of contacting the aqueous feed with a bed of silica gel prior to contact with the adsorbent is to be tested, a 7 cc silica gel column, through which the feed may be passed, is the means provided. The effect of sodium silicate in the feed may be tested simply by adding a known quantity of that compound to the feed. The adsorbent chamber effluent can be analyzed on-stream or, alternatively, effluent samples can be collected periodically and later analyzed separately by analytical equipment.

From information derived from the test adsorbent, the effect of the added silica can be rated by a comparison of the concentrations of dissolved silica in the feed water to the adsorbent chamber and the water comprising the effluent of the adsorbent chamber. If these concentrations are substantially identical, the indication would be that there is no net silica loss from the adsorbent. If the silica concentration of the effluent is greater than that of the feed, the indication would be that the silicon constituent of the crystalline aluminosilicate is dissolving in the aqueous stream.

The following examples are presented to illustrate our invention and are not intended to unduly restrict the scope and spirit of the claims attached hereto.

## EXAMPLE I

The purpose of this Example is to demonstrate that only a silica gel guard bed is effective in preventing silica dissolution of a crystalline aluminosilicate adsorbent. The above described dynamic testing apparatus was used to obtain the data for this Example. The immediately following data is illustrative of the practice of our invention, i.e. the source of silica was 7 cc silica gel column (the temperature of the adsorbent was maintained at 60° C.):

| Total Volume Pumped, Liters | Temp of Si Gel Column, °C. | ppm Si in Feed H <sub>2</sub> O | ppm Si in Eff. H <sub>2</sub> O | 15 |
|-----------------------------|----------------------------|---------------------------------|---------------------------------|----|
| 2.56                        | —                          | 0                               | 15.3                            |    |
| 2.85                        | 34                         | 10.6                            | 14.5                            |    |
| 4.30                        | 32                         | 5.4                             | 15.3                            |    |
| 4.66                        | 40                         | 11.0                            | 15.1                            |    |
| 6.13                        | 42                         | 12.5                            | 16.5                            |    |
| 6.34                        | 46                         | 16.1                            | 16.7                            |    |
| 7.93                        | 50                         | 36.3                            | 34.4                            | 20 |
| 8.34                        | 51                         | 39.5                            | 32.8                            |    |
| 8.54                        | 51                         | 38.7                            | 38.8                            |    |

The next following data was obtained not by the practice of our invention, which utilizes a silica gel guard bed, but with sodium silicate being added to the adsorbent feed to provide a source of silica. Except for the source of silica, all details of operation of the dynamic testing apparatus were unchanged from those used in obtaining the above data:

| Total Volume Pumped, Liters | ppm Si in Feed H <sub>2</sub> O | ppm Si in Eff. |
|-----------------------------|---------------------------------|----------------|
| 1.69                        | 15                              | 14.7           |
| 2.87                        | 15                              | 17.9           |
| 3.09                        | 15                              | 24.8           |
| 3.38                        | 15                              | 25.4           |

During the same test run, the source of silica was switched to a silica gel bed, i.e. in accordance with our invention, and the following additional data was obtained:

| Total Volume Pumped, Liters | ppm Si in Feed H <sub>2</sub> O | ppm Si in Eff. |
|-----------------------------|---------------------------------|----------------|
| 5.06                        | 14.4                            | 15.7           |
| 6.20                        | 13.4                            | 15.7           |
| 6.52                        | 14.0                            | 16.7           |

It can be seen from all of the above data that when a silica gel guard bed is used, in accordance with our invention, the concentration of the silica in the feed water to the adsorbent tends to be substantially the same as in the adsorbent chamber effluent water. This indicates that little, if any, silicon constituent is removed from the adsorbent. On the other hand, when the use of a source of silica other than silica gel is attempted, the concentration of the silica in the effluent is consistently greater than that in the feed, which indicates a net loss in the silicon constituent and ultimate dissolution of the crystalline aluminosilicate adsorbent.

## EXAMPLE II

The purpose of this example is to demonstrate that our invention is most effective when the adsorbent temperature is not greater than about 65° C. Again, the apparatus used to obtain the data for this example was

the dynamic testing apparatus as hereinbefore described. The following data was obtained:

| 5 | Total Volume Pumped, Liters | ppm Si in Feed H <sub>2</sub> O | ppm Si in Effluent | Temp °C. of Adsorbent |
|---|-----------------------------|---------------------------------|--------------------|-----------------------|
|   | 2.4                         | 0                               | 15                 | 75                    |
|   | 17.2                        | 0                               | 12.2               | 75                    |
|   | 36.4                        | 0                               | 10.3               | 75                    |
|   | 46.1                        | 0                               | 8.9                | 75                    |
|   | 74.9                        | 0                               | 6.1                | 68                    |
|   | 84.6                        | 0                               | 4.7                | 65                    |
|   | 131.8                       | 0                               | 7.1                | 72                    |
|   | 176.4                       | 0                               | 8.0                | 74                    |
|   | 200.1                       | 8.9                             | 12.2               | 74                    |
|   | 222.5                       | 9.9                             | 16.9               | 70                    |
|   | 290.1                       | 13.6                            | 16.0               | 76                    |
|   | 318.6                       | 2.4                             | 4.7                | 76                    |
|   | 357.3                       | 9.2                             | 8.9                | 65                    |
|   | 386.2                       | 9.9                             | 9.9                | 65                    |
|   | 405.4                       | 11.8                            | 11.8               | 65                    |
|   | 415.1                       | 11.8                            | 11.8               | 66                    |
|   | 424.7                       | 6.6                             | 6.1                | 54                    |
|   | 434.3                       | 14.6                            | 12.2               | 54                    |
|   | 453.6                       | 11.0                            | 11.3               | 54                    |
|   | 482.9                       | 11.8                            | 12.0               | 56                    |

It is apparent from the foregoing data of this example that only when the temperature of the adsorbent is less than about 65° C. will the concentration of the silica in the feed water to the adsorbent be substantially the same as in the adsorbent chamber effluent water. It is preferred, therefore, that in the practice of our invention the adsorbent temperature be maintained below about 65° C. to avoid the dissolution of the crystalline aluminosilicate.

We claim as our invention:

1. In a process for the separation of a component from a feed mixture comprising an aqueous solution comprising a mixture of saccharides components by contacting an aqueous solution comprising a mixture of saccharide components with an adsorbent comprising a crystalline aluminosilicate exhibiting an adsorptive selectively towards said component thereby selectively adsorbing said component from said mixture, maintain said adsorbent at a temperature of less than 65° C., and thereafter recovering said adsorbed component by elution with an aqueous desorbent, the silicon constituent of said crystalline aluminosilicate tending to dissolve in said solution resulting in the undesirable disintegration of said crystalline aluminosilicate, the improvement which comprises contacting said feed mixture or said desorbent with a bed of silica gel prior to contacting said feed or said desorbent with said adsorbent, thereby effecting a substantial reduction in the extent of dissolution of said silicon constituent and the extent of said disintegration of said crystalline aluminosilicate in said adsorbent.

2. The process of claim 1 further characterized in that said adsorbent incorporates therein a binder material comprising amorphous silica-alumina or alumina.

3. The process of claim 1 further characterized in that said saccharides comprise a mixture of fructose and glucose.

4. The process of claim 1 further characterized in that the pH of said aqueous solution is from about 5.5 to about 7.5.

5. The process of claim 1 further characterized in that said crystalline aluminosilicate is selected from the group consisting of X zeolites and Y zeolites.

6. The process of claim 5 further characterized in that said aluminosilicate contains cations at exchangeable cationic sites selected from the group consisting of alkali metals and alkali earth metals.

\* \* \* \* \*